

July 8, 1952

W. M. BUSKES ET AL

2,602,742

SENSITIZED SHEETS PROVIDED WITH A SCREEN

Filed Oct. 24, 1946



FIG.1



FIG.3



FIG.4



FIG.5



FIG.6

FIG.8



FIG.7

FIG.9



WILLEM MARIE BUSKES; THEODORUS PETRUS WILHELMUS SANDERS;  
MATHEUS MARINUS PAULUS VALLEN; KAREL MARIA HUTGENS

BY *Hammond & Littell*, ATTORNEYS

## UNITED STATES PATENT OFFICE

2,602,742

## SENSITIZED SHEETS PROVIDED WITH A SCREEN

Willem Marie Buskes, Velden, and Theodorus Petrus Wilhelmus Sanders, Matheus Marinus Paulus Vallen, and Karel Maria Hutgens, Venlo, Netherlands, assignors to Chemische Fabriek L. van der Grinten, Venlo, Netherlands, a company of the Netherlands

Application October 24, 1946, Serial No. 705,310  
In the Netherlands November 1, 1945

26 Claims. (Cl. 95-8)

1

This invention relates to sensitized sheets provided with a covering screen to be used in the production of screen reflex copies in the positive diazo process.

It is often necessary for the screen-pattern in such screen covered sheets, particularly those with a fine screen structure, to be in close proximity to the sensitized layer, as for example, with the use of diffused light in screen-reflectography. In such cases the screen-pattern calls for greater accuracy and covering than is obtained in ordinary printing technique, high printing, deep printing and flat printing. While this accuracy and covering is obtained with certain types of photographically produced screen-patterns, these on the whole are expensive and offer a very limited choice as to the substances capable of forming the covering portions (light obstructing portions) of the screen-patterns.

This invention provides relatively inexpensive transparent light-sensitive sheets formed with an integral screen, for use in positive diazotype reflectography processes, which meet high requirements. The screen pattern of these sheets consists solely of portions that are substantially impervious to light to which the sensitized layer is sensitive, alternating with portions that are substantially entirely pervious to such light, i. e., without intermediate graded transitions.

According to the invention the screened sensitized sheets are so constituted that the screen-pattern is arranged in the immediate vicinity of the sensitized layer and that the substance constituting the covering (light-obstructing) portions of the screen is deposited in cavities in the sheet.

This permits of a wide choice in the selection of substances for the covering portion, as a result of which, particularly effective screened sheets are possible—as will appear from the examples.

In one embodiment of the invention, which provides the desired close contact between screen-pattern and sensitized layer, the cavities containing the substances constituting the covering portions are formed in the sensitized layer itself. This construction is specially adapted for use in screen-reflectography and is, generally speaking, cheap. The copy obtained with such a sheet has a relief surface which, provided it possesses sufficient fineness of structure, has the advantages of a dull surface (being less glossy and better suited to writing).

One method of obtaining a screen pattern for the sensitized sheets, according to this inven-

tion, is by producing, either in the sheet itself or, where the sheet consists of more than one layer, in one of its component layers, a relief pattern of the desired screen form and in filling the formed cavities of this pattern with the covering substance and removing the excess of this substance by wiping it off, i. e., by doctoring, sweeping or rubbing it off, for example by means of a doctor blade. This relief pattern may be obtained by subjecting the sheet to the action of a press or mould where the sheet is itself sufficiently plastic or becomes plastic e. g. under heat (by heating to a certain temperature), or by casting it on such mould; the press or mould forming the counterpart of the desired pattern (cavities) to be produced in the sheet. As a filler, i. e. the covering substance for the cavities in this relief pattern, pigments, colouring matters, mixtures with colouring matter, carbon black, barite, zinc white and the like may be employed. A covering substance may also be selected which does not absorb visible light but does absorb e. g. ultra-violet light, or the substance may be such that when subjected to an after-treatment, which the image formed on the sensitized layer normally undergoes, it loses its absorptive power or its covering power. Preferably the covering substance is so chosen that it partly or entirely derives its covering power from the finely divided condition in which it is used, and is a substance which is soluble in the liquid with which the copy is afterwards to be treated. In this form of the invention, the cavities must, of course, be accessible to the liquid.

A particularly suitable construction is that in which a sensitized layer is used which, after exposure, requires a treatment with liquid, e. g. a diazotype layer wherein development is effected by covering it with a thin layer of the developer, and in which the cavities are formed in the sensitized layer itself, while the covering substance is soluble in the after-treatment liquid, e. g. the diazotype developer. It is obvious that the covering filler substance should be suitable as regards the sensitized layer, the things with which it comes into contact during processing, the ultimate image, etc. The substance selected as filler should, of course, not lose its covering power too quickly, e. g. under the influence of moisture.

If the covering substance employed is not of such a nature that it can be removed by dissolution, for instance in an after-treatment liquid, it generally should be removable after exposure, 55 in some other way. In some cases its removal

may be effected by stripping off a skin, or sometimes a brushing treatment may be employed. The latter method of removing the filling from the cavities is not entirely satisfactory, besides being difficult to carry out and far from clean.

It has now been found that certain of these difficulties may be obviated by imparting such a degree of cohesion to the particles of the covering screen portions that it will be possible to remove the covering substances, substantially in their entirety, from the cavities. Care should be taken in such a case that the attachment of the coherent screen portions to the bottom and sides of the cavities is not too great.

The desired degree of cohesion between the particles can be obtained by using a suitable amount of a binding agent. A simple way to attain this is to mix, for instance, the paste of the covering substance in e. g. toluene (see Example 3) with a substance like rubber, in such a quantity that, after the toluene has evaporated, the covering portions form a more or less soft, as it were sintered (caked), mass in the cavities. These coherent parts can readily be removed from the cavities in a considerably cleaner way by the method of Example 3 than when the particles possess little, if any cohesion. It has been found that it is possible to select the binding agent and the amount of it in such a manner that the cohering screen portions can be removed very simply, quite cleanly and even in dry condition with the aid of an adhesive surface, for instance dry adhesive paper, adhesive ribbon or the like; to effect this, it is of course necessary for the coherent screen portions to attach themselves adequately to the adhesive surface used.

It is also possible to provide the cavities with coherent covering parts by filling them with a liquid and subsequently passing the foil under a doctor knife, the said liquid being one which, upon solidifying or drying the mass, will form a coherent coating (e. g. of crystals). It is also possible to proceed according to the method of Example 3 and thus obtain a filling without cohesion, followed by impregnation with a liquid which, upon solidifying or drying, supplies the required cohesion.

By repeating the filling and doctoring process more than once it is also possible to arrange different types of fillings in layers, one on top of the other. Thus the bottommost layer in contact with the bottom of the cavity may be one that adheres but slightly thereto, whereas the layer supplied last (the top layer) may be one having a great adhesive power with respect to the adhesive surface to be applied when removing the covering screen portions from the sheet.

Provided one of the layers supplied, for example the last, is sufficiently pervious to the active light and provided it does not attach itself too much to the uncovered tops, this layer, if desired, need not be subjected to a wiping off operation, e. g. by the action of a doctor knife; it will then form a coating extending also over the elevated parts between the cavities proper, thus imparting cohesion of a covering screen portion with the adjacent covering screen portions. This form of the invention is particularly suitable for the removal of the screen with the aid of an adhesive surface, care being taken to ensure that the topmost layer adheres sufficiently to the adhesive surface applied.

For de-screening the sheet with the aid of an adhesive surface, the latter must be of such a nature that the degree of adhesion of the screen

components to the sensitized sheet is smaller than their degree of adhesion to the adhesive surface. In this connection it is observed that in respect of this method of screen-removal words like "adhesive surface," "adhesive power" and the like, are to be taken in a wide sense. Thus, the conception "adhesive surface" e. g. also includes a so-called vacuum surface or a combination of a vacuum and an adhesive surface. "Adhesive power" for instance also comprises the magnetic force acting on screen portions consisting of iron or of a mixture containing a sufficient amount of iron.

When removing a screen skin, de-screening with the aid of an adhesive surface is of particular importance when such screen skins are very thin and weak, i. e. when they have a weight or less than approximately 20 g. per m.<sup>2</sup>.

In many cases the screen can be removed mechanically.

The invention will be elucidated with reference to the drawings and the examples.

In the accompanying drawings:

Fig. 1 is a part sectional view showing a surface configuration for the drum of Fig. 2.

Fig. 2 is a sectional diagram showing a machine for the production of the sheet.

Fig. 3 is a sectional view illustrating a sensitized sheet prepared for being used in the invention to build up the screened sensitized sheet.

Fig. 4 is a sectional view of a complete sensitized sheet on the drum surface according to the invention.

Fig. 5 is a sectional view of a complete sensitized sheet produced by the surface of Fig. 2, after having been taken from the drum.

Figs. 6 and 8 are perspective views showing different matrices.

Figs. 7 and 9 are perspective views showing the resulting screen patterns.

Figs. 10 and 11 are sectional diagrams of devices suitable for de-screening a sensitive sheet.

Referring now to Figs. 1 and 2, 1 indicates a rotating drum having a metal surface in which are formed a series of grooves 2. The drum 1 as it rotates dips into a trough 3 containing a solution 4 so that the surface of the drum on leaving the trough 3 is coated with a film of the solution. As the drum continues to rotate, the film is subjected to the drying action of a heater 5 and the film dries into a thin skin indicated at 6 in Fig. 4 having a continuous series of cavities. When the skin 6 reaches a point opposite the roller 7, a mixture 40 constituting the covering substance is applied to the surface of the skin on the drum so as to fill up the cavities therein. On leaving the roller 7 the covering substance which has been applied to the surface of the drum is subjected to the action of a doctor knife 8 and thence to the drying action of another heater 9. The covering substance which fills the cavities in the skin 6 is indicated at 10 in Fig. 4 and now the drum layer has applied to it the sensitized material. This is carried out by means of a strip of cellulose acetate film 14 (Fig. 3) which travels over rollers 11 and 11' with the sensitized surface 15 innermost, and shortly prior to entering into contact with the drum 1 the sensitized strip of film 14—15 has applied to it a coating 16 (Fig. 3). This coating consists of an adhesive so as to unite the sensitized strip to the covered skin 6—10. By means of a heater 12, heat is applied to the surface of the drum, causing the skin 6—10 to adhere to the adhesive 16 on the film strip and the multi-layered composite strip now leaves

## 5

the drum and passes away over the roller 11 in the direction of the arrow 13. Thus a complete sensitized sheet as represented in Fig. 5 is obtained.

In Fig. 10, 100 is a roller on which a roller 22 exercises a certain amount of pressure. 23 is a frame parallel to the roller 100 and extending over its entire length. 24 is a roll of adhesive paper. When the apparatus is in operation, the adhesive paper 25 will move in the direction of the arrows from roll 24 by way of cylinder 100 and frame 23 to roll 26, where it is re-rolled. The roller 100 is rotated by means of a crank, not represented, for instance by hand, and the roll 26 may be driven by means of friction so as to unwind the adhesive strip from roll 24 which is checked. The adhesive paper 25 consequently runs through the machine under tension. In passing over the roller 100 it has its adhesive side uppermost. When a sensitized sheet 27, suitable for the purpose and provided with a screen, is passed in the same direction with the screen side directed downwards, between the rollers 100 and 22, it will unite with the adhesive paper at the point of passage between the said cylinders and together therewith proceed on its way to the edge 28 of the frame 23. Here the adhesive paper makes a sharp turn downwards, while the sensitized sheet continues straight on (as a rule it is stiff enough to do this). If their degree of adhesion to the sensitized sheet is smaller than their adhesion to the adhesive surface, the covering screen portions will adhere to the strip and be carried along on the latter; in this manner the screen is removed from the sensitized sheet. After that, the latter can be subjected to the usual after-treatment, for example in the case of a diazotype sheet, a half-wet or dry developing process. The de-screening apparatus can be coupled with a developing-apparatus.

Referring to the modification as shown in Fig. 11, the lowermost cylinder 100 is replaced by a perforated cylinder 35, in which is a stationary hollow cylinder 29 having an interior partition 30 and slots 31 and 32, extending over the entire length of the cylinder. On one side of the partition 30, there is a chamber 33 and on the other side a chamber 34. These chambers are closed at one end, the other end being connected to an air-pump, pumping the air from 33 to 34. The air consequently streams in through 31 and out again through 32. Around this cylinder 29 is the perforated cylinder 35 which is mounted so that it rotates in the direction of the arrow. The cylinder 22 exerts pressure on 35. The outer surface of 35 may be adhesive. After an image has been formed, the screened sensitized sheet 27 with the screen skin directed downwards, is introduced between cylinder 22 and cylinder 35, moves in the direction of the arrow, is caught by the suction at 31 and stuck on the surface of 35, after which it is lightly loosened near 38 by means of a point or a narrow blade-shaped object 36 and conducted farther (e. g. by hand) in the direction of the arrow. When the adhesion of the screen skin to the wall 35 at point 38—which adhesion is due to the sucking and/or adhesive power of the said wall—is greater than its adhesion to the sensitized sheet, the screen skin will peel off and continue moving with the wall 35 until it is blown off by the air-stream coming from the slot 32.

## Example 1

Referring to Figs. 1-5 a skin may be formed

## 6

from a solution of nitro-cellulose in acetone, which is placed in the bath 3 while the covering substance applied at 7 consists of carbon black in a 1% solution of gum arabic. The acetyl cellulose film 14, whose thickness is in accordance with 80 g. per m.<sup>2</sup> is superficially saponified and then sensitized, to form layer 15, with a solution of 5% p-diazoethylbenzylaniline chloride,

1% alum

2% thiourea

10% ethyl alcohol

As described above the sensitized film 14 with its sensitized side towards the cylinder 1 is united by means of an adhesive layer of rubber latex 16 to the skin 6, said skin 6 and filling 10 constituting the covering screen.

The product thus obtained is shown in section in Fig. 5. In practice the adhesive layer 16 is negligibly thin. It forms together with the layer 6 and the filling 10 (in closed cavities) a skin that can be stripped from the sensitized sheet 14-15.

The product is laid with its lower side on an original and is exposed through 6. There is obtained a screen reflex copy, which after stripping off the skin consisting of 6, 10 and 16, is developed by applying to layer 15 a film of developer composed as follows:

30 0.8% phloroglucinol  
0.8% resorcinol  
3% sodium carbonate  
6% sodium thiosulphate  
2% thiourea  
35 1% rhodanide of potassium  
0.2% of the sodium salt of isopropyl naphthalene sulphonic acid

## Example 2

40 The same processing as in Example 1 is followed, but the film is sensitized with 1-diazo-3-chloro-4-dimethylamino-benzene, and the covering substance applied at 7 (Fig. 2) consists of a paste of carbon black in water mixed with a little alcohol and gum arabic. This again produces a screened diazotype sheet or film of the type shown in section in Fig. 5, with a screen-pattern only consisting of substantially light impervious covering portions (substantially opaque areas), adjacent to portions pervious to light (substantially transparent areas), without intermediate graded transitions and suitable for screen-reflectography. The covering portions occupy approximately 80% of the surface and the period of the screen-pattern is approximately 75 m. $\mu$ . Since the layer 16 is extremely thin (much thinner than proportionally drawn in Fig. 5), there is—and this is of great importance in screen-reflectography—close contact between the portions 45 10 (in closed cavities) and the sensitized layer 15. After exposure in contact with an original as in screen-reflectography, the screen skin 6-10-16 is stripped off and the sheet is developed. The reflex copy obtained is suitable for being re-copied.

## Example 3

An acetyl cellulose film of 70 g. per m.<sup>2</sup> is soaked a little on one surface by means of acetone. This surface is pressed against a relief mould as shown in Fig. 6 with depressions having the following dimensions: 30 x 30 $\mu$ , depth 15 $\mu$ , period 80 $\mu$ . The surface of the film is thus formed with the pattern of Fig. 7. It is saponified and sensitized as in Example 1. The cavities 20 are filled up with

a paste consisting of carbon black and toluene and then passed under a doctor knife or other suitable wiping device. The heights 21 remain pervious to light. After drying the sheet thus screened, it is exposed over an original in a manner normal in screen-reflectography, and treated by brushing with the same developer as in Example 1. The carbon black constituting the screen is thus removed from the open cavities between the parts 21, while the image appears at the same time. Instead of using carbon black, other covering substances, such as barite, titanium-dioxide or others may be employed.

If instead of a paste of carbon black and toluene for the covering substance, a paste consisting of finely divided thiourea and toluene or ground thiourea-powder is used, then it is not necessary to brush with the developer and it is sufficient to apply a thin (in this case not too thin) layer of developer. The thiourea dissolves by this treatment, thus becoming transparent, and does not again become a covering substance in drying. A sufficiently fine division of thiourea can be obtained by grinding, e. g. with toluene in a colloid-mill. In a similar way it is possible, of course, to apply numerous other soluble substances such as urea, thiourea, potassium oxalate as the covering substance within the spirit of the invention.

#### Example 4

In the manner described in Example 3 a screened sensitized sheet is made on a relief as shown in Fig. 8 and having the following dimensions: width of the channels  $5\mu$ , depth  $8\mu$ , period  $80\mu$ . In this manner a relief formation is obtained as shown in Fig. 9. The side carrying the carbon black screen, it is now treated with a solution of 4% acetyl cellulose in acetone, after which it is dried. The covering screen portions thereby acquire such a degree of cohesion that by pressing them, after exposure, on to an adhesive layer of latex, they remain firmly affixed to the latter. Thus, upon separating the sheet from the adhesive layer, the screen is removed from the sheet.

It is also possible to proceed in the following way: The saponified sensitized sheet provided with the relief, is treated with a 3% solution of acetyl cellulose in acetone, passed under a doctor knife and dried. Thereupon, according to the method of Example 3, carbon black is introduced into the cavities by rubbing into them a paste consisting of 10% of carbon black and 0.8% of colophony in toluene, after which the sheet is dried and passed under a doctoring or wiping-off device. The treatment is subsequently repeated with a 3% solution of acetyl cellulose in acetone, and the sheet again passed under the doctoring or wiping-off device and dried. When the screened sheet thus obtained is immersed in the developer of Example 1, to which a slight amount of acetone is preferably added, the covering screen portions will become detached and by rubbing the surface lightly, for instance with a bit of wadding, can be removed from the cavities, without, to any appreciable extent, impurifying the liquid by loose carbon black particles. In this way considerably cleaner work is obtained than when working without the treatments with acetyl cellulose. Instead of acetyl cellulose also substances like ethyl cellulose can be used.

#### Example 5

The relief of a sensitized sheet as described in Example 4 is filled with toluene in which 35%

of 2,4,6-trinitrotoluene is dissolved and 10% of carbon black is suspended. The sheet is subsequently dried and passed under a doctoring or wiping-off device. Instead of 2,4,6-trinitrotoluene, it is possible to use 1,3,5-trinitro benzene, 1,3-dinitrobenzene, -naphthalene and the like. By immersing the sheet in the developer of Example 1 and rubbing it gently, the covering screen portions will be removed satisfactorily in large pieces. It is also possible to remove the screen by means of an adhesive layer. The carbon black may be replaced by 3.5% of the dyestuff No. 28 from Schlutz's Farbstofftabellen 1931, which dyestuff dissolves in toluene.

#### Example 6

The relief of a sensitized sheet as described in Example 4 is filled with toluene, containing 35% of 2,4,6-trinitrotoluene and 4% of carbon black, passed under a doctoring or wiping-off device and dried. This treatment is repeated with a similar paste, but now with the addition of 2% of rubber. This sheet can be de-screened by means of an adhesive layer having an adhesive power slightly smaller than in the case of Example 5.

#### Example 7

The relief of a sensitized sheet as described in Example 4 is treated with a paste of barium sulphate pigmented with sulphide of lead in benzene, in which 2% of rubber is dissolved; passed under a doctor knife and dried. The screen can very well be removed with the aid of an adhesive layer, but the covering screen portions can also be successfully removed in their entirety in the developer according to Example 1, without loose particles impurifying the developer; the detached screen particles settle satisfactorily.

#### Example 8

In the manner described in Example 3 a sensitized sheet, screened with carbon black is made on a relief according to Fig. 1 having dimensions like those specified in Example 4. It is subsequently treated on the screen side with a solution of 20% of Canada balsam in toluene, passed under a doctor knife and dried. The sheet can be de-screened by means of an adhesive layer. If the Canada balsam had been applied to the cavities together with the carbon black, the removal of the covering screen portions would have been much more difficult or even entirely impracticable.

#### Example 9

An acetyl cellulose film of 80 g. per m.<sup>2</sup> is softened a little on one surface by means of acetone. This surface is pressed against a relief as shown in Fig. 8, having the dimensions indicated in Example 4. The surface of the film will now take the form of Fig. 9. It is saponified and sensitized with an aqueous solution of:

6% p-diazo-dimethyl-o-chloroaniline-chloride  
2% oxalic acid  
1% phenol  
20% ethyl alcohol

By means of pasting and passing under a doctoring or wiping-off device, the cavities of the relief formation are now filled with a paste consisting of finely divided sulphate of barium and an 0.8% colophony solution in toluene. After drying, a thin layer is applied by means of a 4% solution of acetyl cellulose in acetone, after which the sheet is dried again. The film thus

## 9

screened is subjected to exposure on top of an original according to diazotype reflectography and subsequently its screened side, in an apparatus according to Fig. 10, is guided over an adhesive ribbon, the adhesive surface of which consists of dried rubber latex. The film thus de-screened is developed in ammonia-vapour and can be used for re-copying on positive diazotype-layers.

What we claim is:

1. A sheet suitable for reflectography in the positive diazotype process comprising as a unit a transparent support, a light sensitive diazo layer and a screen the pattern of which is in the immediate vicinity of the sensitive diazo layer and consists only of portions substantially impervious to light to which the diazo layer is sensitive, interspersed with portions that are substantially pervious to this light, without intermediate graded transitions, the substantially impervious portions formed by deposits in cavities present in the sheet, said deposits comprising particles constituting substance substantially opaque to said light in such a state of cohesion that the substantially impervious portions are removable from the cavities substantially as integral bodies, and a thin transparent skin interconnecting adjacent deposits as a collective unit removable from the sheet.

2. A sheet suitable for reflectography in the positive diazotype process comprising as a unit a transparent support, a light sensitive diazo layer and a screen the pattern of which is in the immediate vicinity of the sensitive diazo layer and consists only of portions substantially impervious to light to which the diazo layer is sensitive, interspersed with portions that are substantially pervious to this light, without intermediate graded transitions, the substantially impervious portions formed by deposits in cavities present in the sheet, said deposits comprising particles constituting substance substantially

## 10

an inlaid light screen, and a thin skin of celullosic material transparent to said light overlying the elevations of said layer and united with the tops of said bodies, said bodies moving from said cavities as part of said skin upon stripping said skin from said sheet.

5 5. A screened diazotype sheet material as described in claim 3, said cavities intercommunicating around said elevations and the opaque bodies therein being integrally interconnected.

10 6. A screened diazotype sheet material as described in claim 3, said bodies being deposits of a composition of a finely divided pigment and a binder therefor.

15 7. A screened diazotype sheet material as described in claim 3, said bodies being deposits of a composition of carbon black and a binder therefor.

20 8. A screened diazotype sheet material for positive reflectography, comprising in a unitary flexible sheet structure a sheet of a cellulose ester composition, said sheet being superficially saponified and a saponified side thereof being formed as a depth relief and carrying a light-sensitive diazo layer so that said layer presents a myriad of minute cavities interspersed with elevations, said sheet being transparent to the light to which said layer is sensitive, said cavities being filled with deposits opaque to said

25 light constituting an inlaid light screen, and a thin skin of a celullosic material overlying said elevations and united with said deposits, said skin being transparent to said light and being strippable from said sheet and said deposits moving from said cavities as part of the skin upon stripping the skin.

30 9. A screened diazotype sheet material as described in claim 8, said sheet and said skin, respectively, being made of cellulose acetate compositions.

35 10. A screened diazotype sheet material as described in claim 8, said cavities intercommunicating around said elevations and the opaque

40

said light being inlaid over said films and filling said cavities substantially to the level of said elevations to constitute a light screen, and a thin skin of a cellulosic material transparent to said light overlying said elevations and united with said bodies.

14. A screened diazotype sheet material as described in claim 13, said cavities intercommunicating around the respective elevations and the respective thin film portions therein, also the respective opaque bodies therein, being integrally interconnected.

15. A method of producing a screened diazotype sheet material for positive reflectography which comprises providing a transparent sheet of a cellulose ester composition in a plastic state over one side, impressing said plastic side with a depth relief member having a myriad of minute cavities therein interspersed with minute elevations so as to form a complementary myriad of elevations and cavities over said side, superficially saponifying the impressed side, then applying a light-sensitive diazo layer thereover so that said layer presents a corresponding myriad of elevations and cavities, and applying a cohesive opaque composition over said side so as to fill the cavities of said layer with deposits of such composition and wiping such composition from the elevations of said layer to render the elevations light pervious.

16. A method as described in claim 15, and thereafter applying a solution of a transparent cellulosic composition over said side so as to form a thin skin of such composition overlying the elevations and united with the deposits in the cavities of said layer.

17. A method as described in claim 15, and applying to said side before applying said opaque composition a solution of a cellulosic composition so as to form thin films thereof in the bottoms of the cavities of said layer.

18. In a method as described in claim 15, applying to said side before applying said opaque composition a solution of a cellulose ester composition so as to form thin films thereof in the bottoms of the cavities of said layer, and after applying and wiping said opaque composition applying a solution of a cellulose ester composition over said side so as to form a thin strippable skin overlying said elevations and united with said deposits.

19. Sensitized sheet material for producing positive diazotypes by reflectography comprising, in a unitary flexible sheet structure, a flexible support transparent to the exposing light, a light-sensitive diazo layer over a side thereof, and a light screen the pattern of which overlies and at least nearly contacts the diazo layer to possess substantially complete covering power therefor, the flexible sheet structure comprising a layer adhered to said support and extending over its sensitized side and forming a myriad of minute cavities distributed thereover and said screen pattern consisting of portions substantially opaque to said light formed by deposits filling said cavities and interspersed with portions of the cavity forming layer substantially transparent to said light, without intermediate gradated transitions, at least said deposits being separable from the sheet to render it a screenless exposure.

20. Sensitized sheet material for producing positive diazotypes by reflectography comprising, in a unitary flexible sheet structure, a flexible support transparent to the exposing light, a light-sensitive diazo layer over a side thereof,

and a light screen the pattern of which overlies and at least nearly contacts the diazo layer to possess substantially complete covering power therefor, the flexible sheet structure comprising a myriad of minute cavities distributed over said sensitized side and said screen pattern consisting of portions substantially opaque to said light formed by deposits filling said cavities and interspersed with portions substantially transparent to said light, without intermediate gradated transitions, the cavities holding said deposits being formed by a skin transparent to said light, said skin surrounding said deposits and being joined firmly to said diazo layer yet strippable bodily therefrom to separate the screen from other parts of the sheet.

21. Sensitized sheet material for producing positive diazotypes by reflectography comprising, in a unitary flexible sheet structure, a support transparent to the exposing light, a light-sensitive diazo layer over a side thereof, and a light screen the pattern of which covers the diazo layer and consists only of portions substantially opaque to said light interspersed with portions substantially transparent thereto, without intermediate gradated transitions, the sensitive diazo layer comprising a myriad of minute cavities therein distributed evenly over said sensitized side, said opaque portions being formed by deposits filling said cavities.

22. Sensitized sheet material for producing positive diazotypes by reflectography comprising, in a unitary flexible sheet structure, a support transparent to the exposing light, a light-sensitive diazo layer over a side thereof, and a light screen the pattern of which covers the diazo layer and consists only of portions substantially opaque to said light interspersed with portions substantially transparent thereto, without intermediate gradated transitions, the sensitive diazo layer comprising a myriad of minute cavities therein distributed evenly over said sensitized side, said opaque portions being formed by deposits filling said cavities, and being soluble in a liquid useful for developing said diazo layer, whereby the screen pattern is readily removable from the material after an exposure of the material.

23. Sensitized sheet material for producing positive diazotypes by reflectography comprising, in a unitary flexible sheet structure, a support transparent to the exposing light, a light-sensitive diazo layer over a side thereof, and a light screen the pattern of which covers the diazo layer and consists only of portions substantially opaque to said light interspersed with portions substantially transparent thereto, without intermediate gradated transitions, the sensitive diazo layer comprising a myriad of minute cavities therein distributed evenly over said sensitized side, said opaque portions being formed by deposits filling said cavities, and comprising finely divided particles in a state of cohesion such that the deposits are removable bodily from their respective cavities by a pulling force.

24. Sensitized sheet material for producing positive diazotypes by reflectography comprising, in a unitary flexible sheet structure, a support transparent to the exposing light, a light-sensitive diazo layer over a side thereof, and a light screen the pattern of which covers the diazo layer and consists only of portions substantially opaque to said light interspersed with portions substantially transparent thereto, without intermediate gradated transitions, the sensitive diazo

13

layer comprising a myriad of minute cavities therein distributed evenly over said sensitized side, said opaque portions being formed by deposits filling said cavities, said deposits each comprising a plurality of layers of which at least one is opaque to said light and which cohere to each other under a pulling force more strongly than the bottom layer adheres to the bottom of its cavities.

25. Sensitized sheet material for producing positive diazotypes by reflectography comprising, in a unitary flexible sheet structure, a flexible support transparent to the exposing light, a light-sensitive diazo layer over a side thereof, and a light screen the pattern of which overlies and at least nearly contacts the diazo layer to possess substantially complete covering power therefor, the flexible sheet structure comprising a myriad of minute cavities distributed over said sensitized side and said screen pattern consisting of portions substantially opaque to said light formed by deposits filling said cavities and interspersed with portions substantially transparent to said light, without intermediate gradated transitions, the adjacent deposits being interconnected cohesively by means distinct from and strippable bodily from yet joined firmly to the diazo layer, whereby the opaque deposits are readily separable from other parts of the sheet structure.

26. A screened sensitized sheet material for producing positive diazotypes by reflectography comprising, in a unitary flexible sheet structure, a flexible support of cellulosic material carrying a light-sensitive diazo layer on one side and trans-

14

parent to the light to which said layer is sensitive, said support being formed with a depth relief impression over said one side presenting a myriad of minute cavities interspersed with elevations, said cavities being filled by bodies opaque to said light to constitute an inlaid light screen, the respective bodies and elevations forming a surface parallel to the other side of said support and composed of myriads of distinct areas, respectively, opaque and transparent to said light, without intermediate gradated transitions.

WILLEM MARIE BUSKES.

THEODORUS PETRUS WILHELMUS  
SANDERS.MATHEUS MARINUS PAULUS VALLEN.  
KAREL MARIA HUTGENS.

## REFERENCES CITED

The following references are of record in the  
20 file of this patent:

## UNITED STATES PATENTS

| Number    | Name            | Date          |
|-----------|-----------------|---------------|
| 492,333   | Levy            | Feb. 21, 1893 |
| 2,026,292 | Van der Grinten | Dec. 31, 1935 |
| 2,051,585 | Van der Grinten | Aug. 18, 1936 |
| 2,283,715 | Yanes           | May 19, 1942  |
| 2,303,395 | Schultz et al.  | Dec. 1, 1942  |

## FOREIGN PATENTS

| Number  | Country       | Date          |
|---------|---------------|---------------|
| 15,994  | Great Britain | 1901          |
| 20,046  | Great Britain | 1909          |
| 229,552 | Germany       | Dec. 24, 1910 |